



US005308747A

**United States Patent** [19]

Szajewski et al.

[11] **Patent Number:** **5,308,747**[45] **Date of Patent:** **May 3, 1994**

[54] **PHOTOGRAPHIC SILVER HALIDE MATERIAL COMPRISING TABULAR GRAINS AND POSITIONED ABSORBER DYES**

[75] **Inventors:** Richard P. Szajewski; James P. Merrill; Allan F. Sowinski, all of Rochester, N.Y.

[73] **Assignee:** Eastman Kodak Company, Rochester, N.Y.

[21] **Appl. No.:** 869,987

[22] **Filed:** Apr. 16, 1992

[51] **Int. Cl.:** G03C 1/08

[52] **U.S. Cl.:** 430/507; 430/517; 430/506; 430/522; 430/518

[58] **Field of Search:** 430/507, 517, 506, 522, 430/518

[56] **References Cited**

**U.S. PATENT DOCUMENTS**

4,312,941 1/1982 Scharf et al. .... 430/510  
4,391,884 7/1983 Meyer et al. .... 430/510  
4,439,520 3/1984 Kofron et al. .... 430/503  
4,740,454 4/1988 Deguchi et al. .... 430/567  
4,746,600 5/1988 Watanabe et al. .... 430/505  
4,833,069 5/1989 Hamada et al. .... 430/504

4,855,220 8/1989 Szajewski ..... 430/505  
4,956,269 9/1990 Ikeda et al. ..... 430/507  
5,075,205 12/1991 Inagaki et al. ..... 430/522

**FOREIGN PATENT DOCUMENTS**

0324656 7/1989 European Pat. Off. ....  
1231044 9/1989 Japan ..... 430/522

**OTHER PUBLICATIONS**

Buhr et al., Research Disclosure Item #25330, May 1985, pp. 237-240.

*Primary Examiner*—Charles L. Bowers, Jr.

*Assistant Examiner*—Thomas R. Neville

*Attorney, Agent, or Firm*—Paul A. Leipold

[57]

**ABSTRACT**

A photographic recording material comprising a support bearing at least one photographic layer comprising a sensitized high aspect ratio tabular grain silver halide emulsion and at least one spatially fixed dye layer spatially positioned between said silver halide layer and the upper surface of said recording material, said dye layer comprises a spatially fixed dye that absorbs light in the region of the spectrum to which the silver halide is sensitized.

**11 Claims, No Drawings**

PHOTOGRAPHIC SILVER HALIDE MATERIAL  
COMPRISING TABULAR GRAINS AND  
POSITIONED ABSORBER DYES

TECHNICAL FIELD

This invention relates to photographic materials, elements, and process specifically to materials and elements having tabular silver halide emulsion grains and spatially fixed dyes in a specified spatial arrangement to enable improved sharpness and processes to reveal such an improved image.

BACKGROUND ART

Among the desirable properties of a photographic silver halide recording material is high sharpness. That is, the recording material should enable faithful reproduction and display of both coarse and fine details of the original scene. This combination of properties has proven difficult to achieve in practice.

A general description of the nature of this problem may be found in T. H. James, Ed., "The Theory of the Photographic Process," Macmillan, New York, 1977 and, in particular, at Chapter 20 of this text, pages 25 578-591, entitled "Optical Properties of the Photographic Emulsion" by J. Gasper and J. J. DePalma.

One method of improving sharpness, disclosed at U.S. Pat. No. 4,312,941 and at U.S. Pat. No. 4,391,884, involves the incorporation of a spatially fixed absorber dye in a film layer between the exposing light source and a layer comprising a conventional grain light sensitive silver halide emulsion. In these disclosures, the absorber dye is held spatially fixed either by means of a ballast group or by means of a mordanting material incorporated at a specified position in the film structure. Use of this spatial arrangement of absorber dye and emulsion reduces front-surface halation effects.

U.S. Pat. No. 4,439,520, *inter alia*, discloses the utility of sensitized high aspect ratio silver halide emulsions for use in light sensitive materials and processes. These high aspect ratio silver halide emulsions, herein known as tabular grain emulsions, differ from conventional grain emulsions in many characteristics. One differential characteristic is the relationship between the emulsion grain thickness and the emulsion grain equivalent circular diameter. Conventional grain emulsions tend to be isotropic in shape and, when incorporated in a film structure, tend to be randomly oriented within a particular layer. Tabular grain emulsions however, tend to be anisotropic in shape and, when incorporated in a film structure, tend to align such that their major axis parallels the plane of the film base. This degree of anisotropy is known as the emulsion aspect ratio (AR), typically defined as the ratio of the emulsion grain equivalent circular diameter divided by the emulsion grain thickness. The ability to control emulsion grain thickness and alignment within a film structure can enable the realization of otherwise unattainable degrees of recording material performance.

The optical properties of photographic recording materials incorporating tabular grain emulsions are described in great detail at "Research Disclosure", No. 25330, May, 1985, as are methodologies of specifying particular arrangements of tabular grain emulsions within a film structure and of specifying particular tabular grain emulsion thicknesses so as to enable the attain-

ment of specifically desired properties, such as speed or sharpness in underlying or overlying emulsion layers.

These methods may not prove to be wholly satisfactory. U.S. Pat. No. 4,740,454, for example, discloses that 5 although high frequency sharpness may be attained by the appropriate choice of tabular grain emulsion thickness and placement, this can be at the cost of low frequency sharpness. The term "high frequency sharpness" generally relates to the appearance of fine detail in 10 a scene reproduction, while the term "low frequency sharpness" generally relates to the appearance of clarity or "snap" in scene reproduction. It is understood that the terms "high frequency sharpness" and "low frequency sharpness" are qualitative in nature and that 15 both image frequency, expressed as cycles/mm in the film plane and the image magnification employed in producing a reproduction must be taken into account when specifying such terms. This publication discloses that both high frequency and low frequency sharpness may be simultaneously improved by the incorporation of specific mercaptothiadiazole compounds in combination with tabular grain silver halide emulsions. This practice may not be wholly satisfactory since the incorporation of such silver ion ligands can lead to deleterious effects on film speed and film keeping properties.

In a related area, U.S. Pat. Nos. 4,746,600 and 4,855,220 disclose that unexpectedly large degrees of sharpness can be attained by combining spatially fixed absorber dyes and Development Inhibitor Releasing Compounds (DIR Compounds) in a photographic silver halide recording material. The spatially fixed absorber dye is positioned between an emulsion containing layer and the exposing light source. The materials described in these disclosures incorporate either conventional grain silver halide emulsions or low aspect ratio tabular grain silver halide emulsions. There is no indication of any dependence in film imaging performance on the thickness or spatial positioning of the light sensitive silver halide emulsion grains in these publications.

Again, in a related area, U.S. Pat. No. 4,833,069 discloses that large degrees of sharpness can be attained by simultaneously controlling imaging layer thickness to between 5 and 18 microns and incorporating large quantities, between 15 and 80 mol % of colored cyan dye-forming couplers, known also in the art as cyan dye-forming color masking couplers. This method may not be wholly satisfactory since the use of excessive quantities of color masking couplers can lead to inferior color 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 990

performance of color negative silver halide photographic materials.

A color negative silver halide photographic recording material incorporating conventional grain silver halide emulsions and a quantity of distributed dye sufficient to reduce the speed of a color record by about 50% has been commercially available for many years. Additionally, it has been common practice in the photographic art to commercially provide silver halide photographic recording materials incorporating conventional grain and/or tabular grain silver halide emulsions in combination with soluble dyes sufficient to reduce the speed of a color record by about 10% for purposes related to ease of manufacture. Likewise, color negative silver halide photographic materials incorporating high aspect ratio tabular grain silver halide emulsion with an average grain thickness of circa 0.11 and 0.14 microns in an intermediately positioned layer has been commercially available for many years.

Despite all of this effort, fully adequate degrees of sharpness have not been attained in silver halide photographic materials comprising high aspect ratio tabular grain emulsions. There is a need to provide a silver halide photographic recording material incorporating high aspect ratio tabular grain silver halide emulsions showing excellent sharpness performance.

#### DISCLOSURE OF INVENTION

An object of the invention is to provide sharper photographic images.

It is another object to provide photographic images with more snap.

It is a further object to provide images with improved viewer perceived color rendition.

The objects of the invention are generally accomplished by providing a photographic recording material comprising a support bearing at least one photographic layer comprising a sensitized high aspect ratio tabular grain silver halide emulsion and at least one fixed dye layer spatially positioned between said silver halide layer and the source of the image exposure, wherein said spatially fixed dye absorbs light in the region of the spectrum to which the silver halide is sensitized.

In a preferred embodiment, the improvement of this invention is provided by a photographic recording material comprising a support bearing at least three photographic elements each photographic element being sensitized to different regions of the spectrum;

wherein at least the most light sensitive layer of at least one photographic element comprises a sensitized high aspect ratio tabular grain silver halide emulsion; and

wherein the photographic material comprises at least one additional layer spatially positioned between said high aspect ratio tabular grain silver halide emulsion layer and the source of the image exposure;

wherein at least one said additional layer comprises a spatially fixed dye that absorbs light in the region of the spectrum to which said at least one high aspect ratio tabular grain silver halide is sensitized.

In another preferred embodiment, the improvement of this invention is provided by a photographic recording material as described above wherein more than one of the photographic elements comprise most sensitive tabular grain containing photographic layers and these most sensitive layers comprise a sensitized high aspect ratio tabular grain silver halide emulsions.

In another preferred embodiment, the improvement of this invention is provided by any of the photographic recording materials as described above wherein the photographic material additionally comprises a DIR compound.

In an especially preferred embodiment, the improvement of this invention is provided by any of the photographic recording materials as described above wherein the majority of the photographic layers comprise sensitized high aspect ratio tabular grain silver halide emulsions and spatially fixed dyes are located nearer the surface of the element than the correspondingly sensitized emulsion layer.

#### MODES FOR CARRYING OUT THE INVENTION

This invention has many advantages over prior photographic elements. The invention allows the effective use of the speed advantages of tabular silver halide grains with very good sharpness of images. Surprisingly the use of the spatially fixed absorber dyes in the layer above emulsions sensitive to the color absorbed by the dyes provides improved sharpness with only a small loss in speed. Prior to this invention it had not been realized that light reflection and scattering were a particular problem in the tabular grains, as they were thought to have less light scattering than three-dimensional grains. The improvement obtained by this invention may be achieved without interference with the composition of the silver halide emulsion grains, thereby decreasing the possibilities of reaction with the emulsion layers. These and other advantages of the invention will be apparent from the detailed description below.

In a photographic material the "most sensitive layer" in an element is the layer that comprises the silver halide most sensitive to the spectral region to which the element as a whole is sensitized.

In performing the invention, it is necessary that the spatially fixed dye be positioned between the silver halide emulsion layer whose sharpness is intended to be improved and the upper surface of the photographic element. As used herein, the term "upper surface" or top refers to the surface directed toward the exposure light, while the lower portion or bottom of the photographic element is that portion towards the base and away from the direction of exposure. The spatially fixed dye absorbs the same color light as the silver halide emulsion whose improvement in sharpness is intended.

In other words, if a tabular silver halide emulsion is in the yellow layer which is sensitive to blue light, then the spatially fixed dye also needs to absorb blue light in order to effect the improvement in sharpness of the blue layer. Also, if improvement in the cyan layer which is sensitive to red light is desired, then the spatially fixed dye needs to absorb red light and be placed above (nearer the upper surface) than the cyan tabular emulsion layer.

The spatially fixed dye may be placed in inner layers or emulsion layers or in an overcoat layer, as long as it is above the tabular emulsion layer whose improvement in performance is intended. In a preferred embodiment of the invention, spatially fixed dyes sensitive to red, blue, and green are all placed in a layer above all of the emulsion layers.

As set forth the use of the invention relating to spatially fixed dyes may also be combined with other improvements in a photographic element involving diffus-

ible dyes that also are absorbing of red, green, and blue and with particularly preferred silver halide emulsions that result in superior performance.

The photographic materials of this invention can be either single color or multicolor materials. Multicolor materials typically contain dye image-forming elements sensitive to each of the three primary regions of the spectrum. In some cases the multicolor material may contain elements sensitive to other regions of the spectrum or to more than three regions of the spectrum. Each element can be comprised of a single emulsion layer or of multiple emulsion layers sensitive to a given region of the spectrum. The layers of the material, including the layers of the image-forming elements, can be arranged in various orders as known in the art.

A typical multicolor photographic material comprises a support bearing a cyan dye image-forming element comprising at least one red-sensitive silver halide emulsion layer having associated therewith at least one cyan dye-forming coupler, a magenta image forming element comprising at least one green-sensitive silver halide emulsion layer having at least one magenta dye-forming coupler and a yellow dye image-forming element comprising at least one blue-sensitive silver halide emulsion layer having associated therewith at least one yellow dye-forming coupler. In some instances it may be advantageous to employ other pairings of silver halide emulsion sensitivity and dye image-forming couplers, as in the pairing of an infra-red sensitized silver halide emulsion with a magenta dye-forming coupler or in the pairing of a blue-green sensitized emulsion with a coupler enabling minus-cyan dye formation. The material can contain additional layers, such as filter layers, interlayers, overcoat layers, subbing layers, and the like. The layers of the material above the support typically have a total thickness of between about 5 and 30 microns. The total silver content of the material is typically between 1 and 10 grams per m<sup>2</sup>.

The sensitized high aspect ratio tabular grain silver halide emulsions useful in this invention include those disclosed by Kofron et alia in U.S. Pat. No. 4,439,520 and in the additional references cited below. These high aspect ratio tabular grain silver halide emulsions and other emulsions useful in the practice of this invention can be characterized by geometric relationships, specifically the Aspect Ratio and the Tabularity. The Aspect Ratio (AR) and the Tabularity (T) are defined by the following equations:

$$AR = \frac{\text{Equivalent Circular Diameter}}{\text{Thickness}}$$

$$T = \frac{\text{Equivalent Circular Diameter}}{\text{Thickness} \times \text{Thickness}}$$

where the equivalent circular diameter and the thickness of the grains, measured using methods commonly known in the art, are expressed in units of microns.

High Aspect Ratio Tabular Grain Emulsions of this invention are preferred to have an AR greater than 10. These useful emulsions additionally can be characterized in that their Tabularity is greater than 25 and they are preferred to have a tabularity greater than 50.

Examples illustrating the preparation of such useful emulsions will be shown below.

In the following discussion of suitable compounds for use in the material of this invention, reference will be made to Research Disclosure, December 1989, Item 308119, published by Kenneth Mason Publications,

Ltd., The Old Harbourmaster's 8 North Street, Emsworth, Hampshire PO10 7DD, ENGLAND, the disclosure of which are incorporated herein by reference. This publication will be identified hereafter by the term "Research Disclosure".

The silver halide emulsions employed in the material of this invention can be comprised of silver bromide, silver chloride, silver iodide, silver chlorobromide, silver chloroiodide, silver bromoiodide, silver chlorobromoiodide or mixtures thereof. The emulsions can include silver halide grains of any conventional shape or size. Specifically, the emulsions can include coarse, medium or fine silver halide grains. High aspect ratio tabular grain emulsions are specifically contemplated for at least one layer of the invention elements, such as those disclosed by Wilgus et al U.S. Pat. No. 4,434,226, Daubendiek et al U.S. Pat. No. 4,414,310, Wey U.S. Pat. No. 4,399,215, Solberg et al U.S. Pat. No. 4,433,048, Mignot U.S. Pat. No. 4,386,156, Evans et al U.S. Pat. No. 4,504,570, Maskasky U.S. Pat. No. 4,400,463, Wey et al U.S. Pat. No. 4,414,306, Maskasky U.S. Pat. Nos. 4,435,501 and 4,643,966, and Daubendiek et al U.S. Pat. Nos. 4,672,027 and 4,693,964. Also specifically contemplated are those silver bromoiodide grains with a higher molar proportion of iodide in the core of the grain than in the periphery of the grain, such as those described in G. B. Patent 1,027,146; Japanese 54/48521; U.S. Pat. No. 4,379,837; U.S. Pat. No. 4,444,877; U.S. Pat. No. 4,665,012; U.S. Pat. No. 4,686,178; U.S. Pat. No. 4,565,778; U.S. Pat. No. 4,728,602; U.S. Pat. No. 4,668,614; U.S. Pat. No. 4,636,461; EP 264,954; and U.S. Ser. No. 842,683 of Antoniades et al filed Feb. 27, 1992. The silver halide emulsions can be either monodisperse or polydisperse as precipitated. The grain size distribution of the emulsions can be controlled by silver halide grain separation techniques or by blending silver halide emulsions of differing grain sizes.

Sensitizing compounds, such as compounds of copper, thallium, lead, bismuth, cadmium and Group VIII noble metals, can be present during precipitation of the silver halide emulsion.

The emulsions can be surface-sensitive emulsions, i.e., emulsions that form latent images primarily on the surfaces of the silver halide grains, or internal latent image-forming emulsions, i.e., emulsions that form latent images predominantly in the interior of the silver halide grains. The emulsions can be negative-working emulsions, such as surface-sensitive emulsions or unfogged internal latent image-forming emulsions, or direct-positive emulsions of the unfogged, internal latent image-forming type, which are positive-working when development is conducted with uniform light exposure or in the presence of a nucleating agent.

The silver halide emulsions can be surface sensitized. Noble metal (e.g., gold), middle chalcogen (e.g., sulfur, selenium, or tellurium), and reduction sensitizers, employed individually or in combination, are specifically contemplated. Typical chemical sensitizers are listed in Research Disclosure, Item 308119, cited above, Section III.

The silver halide emulsions can be spectrally sensitized with dyes from a variety of classes, including the polymethine dye class, which includes the cyanines, merocyanines, complex cyanines, and merocyanines (i.e., tri-, tetra-, and poly-nuclear cyanines and merocyanines), oxonols, hemioxonols, styryls, merostyryls, and streptocyanines. Illustrative spectral sensitizing dyes are

disclosed in *Research Disclosure*, Item 308119, cited above, Section IV.

The spatially fixed dyes useful in photographic elements are well known in the art. These spatially fixed dyes are also known as non-diffusible dyes and as anti-halation dyes. The spatially fixed dyes utilized in the invention include dyes and their preparation and methods of incorporation in photographic materials disclosed in U.S. Pat. Nos. 4,855,220; 4,756,600; and 4,956,269, as well as by commercially available materials. Other examples of spatially fixed dyes suitable for the invention are disclosed at Section VIII of *Research Disclosure*, Item 308119.

The spatially fixed dye selected for the invention absorbs light in the region of the spectrum to which the high aspect ratio tabular grain silver halide layer of the invention is sensitized. While the dye will generally absorb light primarily only in that region, dyes that absorb light in broader areas of the spectrum including the region to which the silver halide is sensitized, are also included within the scope of the invention. A simple test as to whether the spatially fixed dye is suitable for the invention is if the speed of the silver halide layer of the invention is less when the dye is present than when it is not, then the dye is within the scope of those useful in the invention.

By spatially fixed, it is meant that substantially none of the dye will migrate out of the layer in which it has been incorporated before the photographic material has been processed.

These dyes may be ballasted to render them non-diffusible or they may be intrinsically diffusible but rendered non-diffusible by use of organic mordanting materials, such as charged or uncharged polymeric matrixes, or rendered non-diffusible by adhesion to inorganic solids such as silver halide, or organic solids all as known in the art. Alternatively, these dyes may be incorporated in polymeric latexes. These dyes may additionally be covalently bound to polymeric materials.

These dyes may retain their color after processing or may change in color, be decolorized or partially or completely removed from the photographic material during processing. For ease of direct viewing or optical printing it may be preferred that the dyes be removed from the material or be rendered non-absorbing in the

visible region during or after processing. During photographic development (generally in high pH, e.g. 9 or above, sulfite containing processing solution), bleaching (in iron containing or persulfate or other peroxy containing solutions at lower pH, e.g. 7 or below) or fixing, the dye may be decolorized or removed from the material. In photographic materials where the image may be electronically scanned or digitally manipulated, the material may or may not retain some degree of coloration depending on the intended use.

The spatially fixed dye may be a diffusible acidic dye that is rendered non-diffusible by incorporating a base group-containing polymeric mordant for the dye at a specified position in the photographic material. Such dyes preferably have a sulfo- or carboxy-group. Useful dyes can be acidic dyes of the azo type, the triphenylmethane type, the anthroquinone type, the styryl type, the oxanol type, the arylidene type, the merocyanine type, and others known in the art. Polymer mordants are well known in the art and are described, for example, in U.S. Pat. Nos. 2,548,564; 2,675,316; 2,882,156; and 3,706,563 as well as in *Research Disclosure*.

The spatially fixed dye may also be a solid particle dispersion of a loaded polymer latex of a dye that is insoluble at coating pH but soluble at processing pH's as described in U.S. Pat. No. 4,855,221—Factor et al.

Additionally, the dye may be a colored image dye-forming coupler as disclosed in *Research Disclosure*, Item 308119, Section VII. The color of such a dye may be changed during processing. The dye may be a pre-formed image coupler dye which would generally remain in the material during processing. The dye may also be a spectral sensitizing dye immobilized by adsorption to chemically unsensitized silver halide. Such a dye would generally be removed from the material during the bleaching or fixing step. It is also preferred to use spatial dyes in hues to match printing compatibility.

It is preferred that such spatially fixed dyes be positioned closer to the image exposure source than the photographic layer comprising a high aspect ratio tabular grain silver halide emulsion sensitized to a region of the spectrum where such dyes absorb light.

Examples of preferred spatially fixed dyes include the dye materials described in the photographic examples illustrating the practice of this invention and include the structures shown below.

CM-1



-continued

MN-1



MM-2



CD-1



MD-1



5,308,747

**11****12**

-continued

YD-1



YD-2



SOL-M1



SOL-C1



-continued



Other useful dye structures include but are not limited to

where

$R_c = -H$  or  $-CH_3$   
and  $R_d = -H$ ;  $-CH_2CH_2OH$ ;  $-CH_2CH_3$ ; or  $-CH_2CH_2NH_2$

Examples of polymer mordants useful in combination with diffusible acidic dyes in elements of the present invention including the following:



Alternatively, it may be desirable to employ anionically charged polymers in combination with diffusible cationic dyes.

The distributed dyes useful in combination with the invention spatially fixed dyes typically may be any of the soluble dyes known in the art as disclosed commercially, in U.S. Pat. Nos. 4,855,220; 4,756,600; and 4,956,269, or at Section VIII of *Research Disclosure* cited earlier.

By distributed, it is meant that quantities of the dye (or a dye combination) which absorbs light in the region of the spectrum to which the high aspect ratio tabular grain silver halide layer of the invention is sensitized are present in several of the layers of the photographic material before the exposure of said material.

It is preferred that such distributed dyes be positioned both closer to, coincident with and further from the image exposure source than the photographic layer comprising a high aspect ratio tabular grain silver halide emulsion sensitized to a region of the spectrum where such dyes absorb light.

These soluble dyes may be diffusible and have the property of distributing within the structure of a photographic material to a greater or lesser extent during a wet coating procedure or during a subsequent curing or storage procedure. Alternatively, these dyes may be added to a photographic material in a subsequent coating, imbibing or like procedure as known in the art. These soluble dyes may additionally be caused to distribute in specific patterns within a photographic material by the addition of mordanting materials in appropriate quantities and positions within the structure of the

photographic material. The mordanting material may be the charged or uncharged polymeric materials described earlier. Alternatively, the distribution of the dye may be controlled by the quantity and disposition of hydrophobic organic materials such as couplers or coupler solvents or absorbent charged or uncharged inorganic materials such as silver halide and the like within the coating structure.

Alternatively, non-diffusible dyes may be employed. 10 These may include any of the non-diffusible dyes previously described. When non-diffusible dyes are employed they may be distributed within a photographic material by addition of a portion of each to the photographic layers as they are coated. However, while it is possible in use of non-diffusible dyes to put them in many layers, it is much preferred to only put the non-diffusible (spatially fixed dyes) into an upper layer of the photographic element.

The dye absorbs light in the region of the spectrum to 20 which the high aspect ratio tabular grain silver halide layer of the invention is sensitized. While the dye will generally absorb light primarily only in that region, dyes that absorb light in other regions of the spectrum as well as the region to which the silver halide is sensitized are also included within the scope of the invention. A simple test as to whether the distributed dye is within the scope of the invention is if the speed of the silver halide layer of the invention is reduced by at least 25 20% by the presence of the distributed dye, then the distributed dye is within the scope of the invention. The greater than 20 percent loss in speed (sensitivity) is acceptable, as there is a great increase in sharpness.

These spatially fixed and diffusible dyes if present 30 may retain their color after processing or may change in color, be decolorized or partially or completely removed from the photographic material during processing. For ease of direct viewing or optical printing it may be preferred that the dyes be removed from the film or rendered non-absorbing in the visible region during or 35 after processing. During photographic development (generally in high pH, e.g., 9 or above, sulfite containing processing solution), bleaching (in iron containing or persulfate or other peroxy containing solutions at lower pH, e.g., 7 or below) or fixing, the dye may be 40 decolorized or removed from the material. In photographic materials where the image may be electronically scanned or digitally manipulated, the material may or may not retain some degree of coloration depending 45 on the intended use.

The distributed dye may be a diffusible acidic dye. 50 Such dyes preferably have a sulfo- or carboxy-group. Useful dyes can be acidic dyes of the azo type, the triphenylmethane type, the anthroquinone type, the styryl type, the oxanol type, the arylidene type, the merocyanine type, and others known in the art.

Specific examples of distributed dyes are shown in the literature cited earlier, in the discussion of spatially fixed dyes and in the examples illustrating the practice of the invention.

The thicknesses of the silver halide emulsions employed in this invention may be advantageously adjusted for the purposes of improving film performance according to principles described in *Research Disclosure*, May, 1985, Item 25330. This disclosure teaches, by extrapolation from the optical properties of silver bromide sheet crystals, that the thicknesses of silver halide emulsions incorporated in specific photographic layers

and sensitized to one spectral region may be chosen to enable either improved speed or improved sharpness behavior in other photographic layers incorporating silver halide emulsions sensitized to different regions of the spectrum. These improvements are said to occur because the light transmission and reflection properties of the silver halide emulsions are controlled in large part by their grain thicknesses. Further discussion on the relationship between the thickness of silver halide crystals and their reflectance properties can be found in *Optics*, by J. M. Klein, John Wiley & Sons, New York, 1960, pages 582 to 585. These disclosures make no teaching about the relationship between the thickness of a silver halide emulsion sensitized to a particular region of the spectrum and the sharpness behavior of a photographic layer or element using such an emulsion.

In another embodiment of the invention has now been found that the sharpness of a photographic element can be unexpectedly improved by setting the thickness of the sensitized high aspect ratio tabular grain emulsion utilized in a most sensitive layer of that element such that the reflection in the region of the spectrum to which that emulsion is sensitized is at a minimum.

It is preferred that the most sensitive layer comprising a high aspect ratio tabular grain silver halide emulsion in which the thickness of said emulsion is chosen so as to minimize reflectance in the region of the spectrum to which the emulsion is sensitized be further from the image exposure source than another most sensitive layer of an element which comprises a high aspect ratio tabular grain emulsion sensitized to a different region of the spectrum.

Thus, to improve sharpness in a blue sensitized element which incorporates a blue sensitized emulsion with a peak sensitivity at about 450 nm used in a most blue sensitive layer, an emulsion grain thickness of between 0.08 and 0.10 microns is preferred. An emulsion grain thickness close to the center of this range, i.e. 0.09 microns is more preferred. An emulsion grain thickness of between 0.19 and 0.21 microns can also be used to advantage in this instance.

In a like manner, to improve sharpness in a green sensitized element which incorporates a green sensitized emulsion with a peak sensitivity at about 550 nm used in a most green sensitive layer, an emulsion grain thickness of between 0.11 and 0.13 microns is preferred. An emulsion grain thickness close to the center of this range, i.e. 0.12 microns is more preferred. An emulsion grain thickness of between 0.23 and 0.25 microns can also be used to advantage in this instance.

In a similar vein, to improve sharpness in a red sensitized element which incorporates a red sensitized emulsion with a peak sensitivity at about 650 nm used in a most red sensitive layer, an emulsion grain thickness of between 0.14 and 0.17 microns is preferred. An emulsion grain thickness close to the center of this range, i.e. 0.15 microns is more preferred. An emulsion grain thickness of between 0.28 and 0.30 microns can also be used to advantage in this instance.

It is straightforward to choose emulsion grain thicknesses to improve the sharpness behavior of emulsions sensitized to other regions of the spectrum or with peak sensitivity at different wavelengths according to this invention by following the disclosed pattern.

Thus, for an infrared sensitized emulsion with peak sensitivity at 750 nm, an emulsion grain thickness of between 0.17 and 0.19 microns would be chosen, while

for a blue-green sensitized emulsion with peak sensitivity at 500 nm, an emulsion grain thickness of between 0.10 and 0.12 microns would be chosen.

When a photographic element is comprised of more than one photographic layer, it is additionally preferred that the thickness of the silver halide emulsions used in such layers be also chosen so as to minimize reflection in the region of the spectrum to which the emulsion is sensitized.

Even when the thickness of a silver halide emulsion employed in a most sensitive layer is not chosen according to this pattern, it may be useful to choose the thickness of an emulsion used in a less sensitive layer according to the disclosed pattern.

It has also been found that both the speed and sharpness of a first photographic element wherein the most light sensitive layer of that first element comprises a high aspect ratio silver halide emulsion whose thickness has been chosen so as to minimize reflection in the region of the spectrum to which that emulsion is sensitized can be unexpected and simultaneously improved when the photographic material additionally comprises a second photographic element sensitized to a different region of the spectrum wherein the most light sensitive layer of said second element is positioned closer to the image exposure source than the most light sensitive layer of said first element and the most light sensitive layer of said second element additionally comprises a high aspect ratio tabular grain emulsion whose thickness is also chosen to minimize the reflectance in the region of the spectrum to which the first element is sensitive.

Thus, to improve speed and sharpness in a red light sensitive element which comprises a high aspect ratio tabular grain silver halide emulsion with a peak sensitivity at about 650 nm used in a most red sensitive layer, in a photographic material comprising a most green light sensitive layer positioned closer to an image exposure source than the most red light sensitive layer, it is preferred to choose the thickness of the sensitized high aspect ratio tabular grain emulsions employed in both of said most sensitive layers to be between 0.14 and 0.17 microns. An emulsion grain thickness close to the center of this range, 0.15 microns is more preferred. An emulsion grain thickness of between 0.28 and 0.30 microns can also be used to advantage in this instance.

Likewise, to improve speed and sharpness in a red light sensitive element which comprises a high aspect ratio tabular grain silver halide emulsion with a peak sensitivity at about 650 nm used in a most red sensitive layer, in a photographic material comprising a most blue light sensitive layer positioned closer to an image exposure source than the most red light sensitive layer, it is preferred to choose the thickness of the sensitized high aspect ratio tabular grain emulsions employed in both of said most sensitive layers to be between 0.14 and 0.17 microns. An emulsion grain thickness close to the center of this range, 0.15 microns is more preferred. An emulsion grain thickness of between 0.28 and 0.30 microns can also be used to advantage in this instance.

In a similar vein, to improve speed and sharpness in a green light sensitive element which comprises a high aspect ratio tabular grain silver halide emulsion with a peak sensitivity at about 550 nm used in a most green sensitive layer, in a photographic material comprising a most red light sensitive layer positioned closer to an image exposure source than the most green light sensitive layer, it is preferred to choose the thickness of the

sensitized high aspect ratio tabular grain emulsions employed in both of said most sensitive layers to be between 0.11 and 0.13 microns. An emulsion grain thickness close to the center of this range, 0.12 microns is more preferred. An emulsion grain thickness of between 0.23 and 0.25 microns can also be used to advantage in this instance.

Other combinations of two or more high aspect ratio tabular grain emulsions sensitized to different regions of the spectrum and employed in different most sensitive layers of different elements can be obviously derived based on the above disclosure and pattern of preferred thicknesses.

It is especially preferred in a photographic material sensitive to three regions of the spectrum to employ sensitized high aspect ratio tabular grain emulsions whose thicknesses are chosen so as to minimize the reflectance in the region of the spectrum to which the emulsion employed in the most sensitive layer positioned furthest from the image source of all of the most sensitive layers is sensitized.

It is straightforward to choose emulsion grain thicknesses to improve the sharpness behavior of emulsions sensitized to other regions of the spectrum or with peak sensitivity at different wavelengths according to this invention by following the disclosed pattern.

Thus, for an infra-red sensitized emulsion with peak sensitivity at 750 nm, an emulsion grain thickness of between 0.17 and 0.19 microns would be chosen, while for a blue-green sensitized emulsion with peak sensitivity at 500 nm, an emulsion grain thickness of between 0.10 and 0.12 microns would be chosen.

When a photographic element is comprised of more than one photographic layer, it is additionally preferred that the thickness of the silver halide emulsions used in such layers be also chosen so as to minimize reflection in the region of the spectrum to which the emulsion is sensitized.

Even when the thickness of a silver halide emulsion employed in a most sensitive layer is not chosen according to this pattern, it may be useful to choose the thickness of an emulsion used in a less sensitive layer according to the disclosed pattern.

The photographic materials of this invention may advantageously comprise Development Inhibitor Releasing Compounds, also called DIR compounds as known in the art. Typical examples of DIR compounds, their preparation and methods of incorporation in photographic materials are disclosed in U.S. Pat. Nos. 4,855,220 and 4,756,600 as well as by commercially available materials. Other examples of useful DIR compounds are disclosed at Section VII of *Research Disclosure*.

These DIR compounds may be incorporated in the same layer as the high aspect ratio emulsions of this invention, in reactive association with this layer or in a different layer of the photographic material, all as known in the art.

These DIR compounds may be among those classified as "diffusible," meaning that they enable release of a highly transportable inhibitor moiety or they may be classified as "non-diffusible" meaning that they enable release of a less transportable inhibitor moiety. The DIR compounds may comprise a timing or linking group as known in the art.

The inhibitor moiety of the DIR compound may be unchanged as the result of exposure to photographic processing solution. However, the inhibitor moiety may

change in structure and effect in the manner disclosed in U. K. Patent No. 2,099,167; European Patent Application 167,168; Japanese Kokai 205150/83 or U.S. Pat. No. 4,782,012 as the result of photographic processing.

When the DIR compounds are dye-forming couplers, they may be incorporated in reactive association with complementary color sensitized silver halide emulsions, as for example a cyan dye-forming DIR coupler with a red sensitized emulsion or in a mixed mode, as for example a yellow dye-forming DIR coupler with a green sensitized emulsion, all as known in the art.

The DIR compounds may also be incorporated in reactive association with bleach accelerator releasing couplers as disclosed in U.S. Pat. No. 4,912,024, U.S. Pat. No. 5,135,839, and in U.S. application Ser. No. 563,725 filed Aug. 8, 1990.

Specific DIR compounds useful in the practice of this invention are disclosed in the above cited references, in commercial use and in the examples demonstrating the practice of this invention which follow. The structures of other useful DIR compounds are shown below.



-continued



-continued



Suitable vehicles for the emulsion layers and other layers of photographic materials of this invention are

described in *Research Disclosure* Item 308119, Section IX, and the publications cited therein.

In addition to the couplers described herein, the materials of this invention can include additional couplers as described in *Research Disclosure* Section VII, paragraphs D, E, F, and G, and the publications cited therein. These additional couplers can be incorporated as described in *Research Disclosure* Section VII, paragraph C, and the publications cited therein.

The photographic materials of the invention may also comprise Bleach Accelerator Releasing (BAR) compounds as described in European Patents 0 193 389 B and 0 310 125; and at U.S. Pat. No. 4,842,994, and Bleach Accelerator Releasing Silver Salts as described at U.S. Pat. Nos. 4,865,956 and 4,923,784 hereby incorporated by reference. Typical structures of such useful compounds include:



Other useful bleach bleaching and bleach accelerating compounds and solutions are described in the above publications.

The photographic materials of this invention can be used with colored masking couplers as described in U.S. Pat. Nos. 4,883,746 and 4,833,069.

The photographic materials of this invention can contain brighteners (*Research Disclosure Section V*), 60 antifoggants and stabilizers (*Research Disclosure Section VI*), antistain agents and image dye stabilizers (*Research Disclosure Section VII*, paragraphs I and J), light absorbing and scattering materials (*Research Disclosure Section VIII*), hardeners (*Research Disclosure Section XI*), plasticizers and lubricants (*Research Disclosure Section XII*), antistatic agents (*Research Disclosure Section XIII*), matting agents (*Research Disclosure Section* 65

XVI), and development modifiers (*Research Disclosure* Section XXI).

The photographic materials can comprise polymer latexes as described in U.S. patent application Ser. Nos. 720,359 and 720,360 filed Jun. 25, 1991, and 771,016 filed Oct. 1, 1991, and in U.S. Pat. Nos. 3,576,628; 4,247,627; and 4,245,036, the disclosures of which are incorporated by reference.

The photographic materials can be coated on a variety of supports as described in *Research Disclosure* Section XVII and the references described therein.

Photographic materials can be exposed to actinic radiation, typically in the visible region of the spectrum, to form a latent image as described in *Research Disclosure*.

ure Section XVIII and then processed to form a visible dye image as described in *Research Disclosure* Section XIX. Processing to form a visible dye image includes the step of contacting the material with a color developing agent to reduce developable silver halide and oxidize the color developing agent. Oxidized color developing agent in turn reacts with the coupler to yield a dye.

With negative working silver halide this processing step leads to a negative image. To obtain a positive (or reversal) image, this step can be preceded by development with a non-chromogenic developing agent to develop exposed silver halide, but not form dye, and then uniform fogging of the element to render unexposed silver halide developable. Alternatively, a direct positive emulsion can be employed to obtain a positive image.

Development is followed by the conventional steps of bleaching, fixing, or bleach-fixing to remove silver and silver halide, washing, and drying.

Typical bleach baths contain an oxidizing agent to convert elemental silver, formed during the develop-

ment step, to silver halide. Suitable bleaching agents include ferricyanides, dichromates, ferric complexes of aminocarboxylic acids, such as ethylene diamine tetra-acetic acid and 1,3-propylene diamine tetraacetic acid as described at *Research Disclosure*, Item No. 24023 of April 1984, Volume 24, Item No. 111-112.

April, 1984. Also useful are peroxy bleaches such as persulfate, peroxide, perborate, and percarbonate. These bleaches may be most advantageously employed by additionally employing a bleach accelerator releasing compound in the film structure. They may also be advantageously employed by contacting the film structure with a bleach accelerator solution during photo-

ture with a bleach accelerator solution during photographic processing. Useful bleach accelerator releasing compounds and bleach accelerator solutions are discussed in European Patents 0 193 389B and 0 310 125A; and in U.S. Pat. Nos. 4,865,956; 4,923,784; and 4,842,994, the disclosures of which are incorporated by reference.

Fixing baths contain a complexing agent that will solubilize the silver halide in the element and permit its removal from the element. Typical fixing agents include thiosulfates, bisulfites, and ethylenediamine tetraacetic acid. Sodium salts of these fixing agents are especially useful. These and other useful fixing agents are described in U.S. patent application Ser. No. 747,895 by Schmittou et al filed Aug. 19, 1991 entitled "Color Photographic Recording Material Processing," the disclosures of which are incorporated by reference.

In some cases the bleaching and fixing baths are combined in a bleach/fix bath.

The following examples illustrate the practice of this invention. They are not intended to be exhaustive of all

possible variations of the invention. Parts and percentages are by weight unless otherwise indicated.

Specific samples of High Aspect Ratio Tabular Grain Silver Halide Emulsions that can be employed to demonstrate the practice of this invention may be precipitated and sensitized according to the following procedures. Silver halide emulsions useful in the practice of the invention are not, however, limited to those specific samples exemplified below.

#### EMULSION PRECIPITATION AND SENSITIZATION EXAMPLE 1

1. Starting kettle: 45° C., 16 g oxidized gelatin (limed ossein gelatin, treated with peroxide to oxidize all methionine groups), 28 g NaBr, 3990 g distilled water, 2 ml of Nalco-2341 antifoam (pBr = 1.29).

2. Nucleation stage:

a. Single jet run@33 ml/min, 0.2164 N AgNO<sub>3</sub>, for two minutes.

b. Continue single jet silver run; raise kettle temperature from 45° C. to 60° C. over 7.5 minutes.

c. Adjust kettle pH with 5 ml of concentrated NH<sub>4</sub>OH (14.8M) diluted to 200 ml with distilled water. Continue single jet silver run throughout this segment for 5 minutes.

d. Stop silver run. Adjust kettle pH to starting value with 3.5 ml of concentrated HNO<sub>3</sub>, diluted to 200 ml with distilled water. Hold for 2 minutes.

e. Add to kettle: 200 g of oxidized gelatin dissolved in 3991 g distilled water at 60° C. Hold 5 minutes.

3. Lateral growth:

Double jet with pBr controlled at 1.82, using 3.0N AgNO<sub>3</sub> and a salt solution which is 2.991M NaBr and 0.033M KI; following to the flow rate profile below:

|              |                    |
|--------------|--------------------|
| 10 minutes   | 20 ml/min          |
| 10 minutes   | 20 to 47 ml/min    |
| 10 minutes   | 47 to 87 ml/min    |
| 11.1 minutes | 87 to 145.9 ml/min |

4. Add to kettle a 292.5 g NaBr and 9.55 g KI dissolved in 535.5 g of distilled water. Hold 2 minutes.

5. Add to kettle 14.3 ml of a solution containing 0.17 mg/ml potassium selenocyanate, diluted to 150 ml with distilled water. Hold 2 minutes.

6. Add 0.316 mole of AgI Lippmann emulsion to kettle. Hold 2 minutes.

7. Single jet silver run with 3N AgNO<sub>3</sub> at 100 ml/min for 10.3 minutes. Reduce silver addition rate to 10 ml/min until kettle pBr reaches 2.50.

8. Wash emulsion to pBr = 3.40 at 40° C. using ultrafiltration, concentrate, add 226 gm of limed ossein gelatin, 80 ml of solution containing 0.34 mg/ml 4-chloro-3,5-xylenol in methanol, chill set, and store.

The resulting emulsion is 4.1 mole % I.

This formula can be used to prepare emulsions typically 0.07 to 0.10 microns thick. Variations which can be made to this formula include changes in nucleation flowrate, the volume and gel concentration in the dump following the precipitation, and lateral growth pBr. The formula may also be scaled-up to produce larger quantities.

Green light spectral sensitizations (per mole of silver):

This procedure is representative of the green light spectral sensitizations on this emulsion type. Variations in sensitizing dye, thiocyanate, finish modifier, chemical sensitizers, and in finish time may be used as known in the art to reach an optimum finish position for a particular emulsion.

the art to reach an optimum finish position for a particular emulsion.

a. Melt emulsion at 40° C. Add 256 g of 12.5% gelatin solution (use limed ossein gelatin) to bring gel content to 78 g/mole silver.

b. Add 150 mg NaSCN. Hold 20 minutes with stirring.

c. Add green light spectral sensitizing dyes at 1.4 mmole dye/mole Ag. Higher or lower mole ratios may be employed in specific sensitizations. Single sensitizing dye or multiple sensitizing dye sensitizations may be employed as known in the art. When multiple dye sensitizations are employed, the dyes may be added together or may be added separately with an optional hold time between additions.

d. Add 3.00 mg of sodium thiosulfate pentahydrate. Hold 2 minutes.

e. Add 1.5 mg of potassium tetrachloroaurate(III). Hold 2 minutes.

f. Add 36.50 mg finish modifier (3-(N-methylsulfonyl)carbamoylethyl benzothiazolium tetrafluoroborate). Hold 15 minutes.

g. Raise melt temperature from 40° to 60° C. over 15 minutes. Hold at 65 degrees for 20 minutes. Cool rapidly to 40 degrees and chill set with stirring.

Red light spectral sensitization (per mole of silver):

This procedure is representative of the red light spectral sensitizations on this emulsion type. Variations in sensitizing dye, thiocyanate, finish modifier, chemical sensitizers, and in finish time may be used as known in the art to reach an optimum finish position for a particular emulsion.

a. Melt emulsion at 40° C. Add 256 g of 12.5% gelatin solution (use limed ossein gelatin) to bring gel content to 78 g/mole silver.

b. Add 120 mg NaSCN. Hold 20 minutes with stirring.

c. Add red light spectral sensitizing dyes at 1.3 mmole dye/mole Ag. Higher or lower mole ratios may be employed in specific sensitizations. Single sensitizing dye or multiple sensitizing dye sensitizations may be employed as known in the art. When multiple dye sensitizations are employed the dyes may be added together or may be added separately with an optional hold time between additions.

d. Add 2.50 mg of sodium thiosulfate pentahydrate. Hold 2 minutes.

e. Add 1.25 mg of potassium tetrachloroaurate(III). Hold 2 minutes.

f. Add 20.0 mg finish modifier (3-(N-methylsulfonyl)carbamoylethyl benzothiazolium tetrafluoroborate). Hold 15 minutes.

g. Raise melt temperature from 40 to 60 degrees over 12 minutes. Hold at 60 degrees for 25 minutes. Cool rapidly to 40 degrees and chill set with stirring.

#### EMULSION PRECIPITATION AND SENSITIZATION EXAMPLE 2A

The preparation of thickened emulsions can be based on the formula given in Emulsion Precipitation and Sensitization Example 1 above. In this example the emulsion sample is precipitated as in Example 1 with the following changes:

The starting kettle temperature is 55° C. and the temperature ramp during step 2a is from 55° to 70° C. The remainder of the make is at 70° C. Limed ossein gelatin was used in place of the oxidized gel in step 2e. The pBr

for the lateral growth step was 1.96 at 70° C. The resulting emulsion was 1.90 microns equivalent circular diameter and 0.139 microns thick.

This procedure is representative of the red light spectral sensitizations on this emulsion type. Variations in sensitizing dye, thiocyanate, finish modifier, chemical sensitizers, and in finish time may be used as known in the art to reach an optimum finish position for a particular emulsion.

a. Melt emulsion at 40° C. Add 256 g of 12.5% gelatin solution (use limed ossein gelatin) to bring gel content to 78 g/mole silver.

b. Add 100 mg NaSCN. Hold 20 minutes with stirring.

c. Add red light spectral sensitizing dyes at 0.9 mmole dye/mole Ag. Higher or lower mole ratios may be employed in specific sensitizations. Single sensitizing dye or multiple sensitizing dye sensitizations may be employed as known in the art. When multiple dye sensitizations are employed the dyes may be added together or may be added separately with an optional hold time between additions.

d. Add 2.00 mg of sodium thiosulfate pentahydrate. Hold 2 minutes.

e. Add 1.00 mg of potassium tetrachloroaurate(III). Hold 2 minutes.

f. Add 20.0 mg finish modifier (3-(N-methylsulfonyl)-carbamoylethyl benzothiazolium tetrafluoroborate). Hold 15 minutes.

g. Raise melt temperature from 40 to 62.5 degrees over 13.5 minutes. Hold at 62.5 degrees for 12 minutes. Cool rapidly to 40 degrees and chill set with stirring.

#### EMULSION PRECIPITATION AND SENSITIZATION EXAMPLE 2B

In another example the emulsion sample is precipitated as in Example 1 with the following changes:

The starting kettle temperature is 50° C. and the temperature ramp during step 2a is from 50° to 65° C. The remainder of the make is at 65° C. Limed ossein gelatin was used in place of the oxidized gel in step 2e. The pBr for the lateral growth step was 2.02 at 65° C. The resulting emulsion was 1.7 microns equivalent circular diameter and 0.145 microns thick.

This procedure is representative of the green light spectral sensitizations on this emulsion type. Variations in sensitizing dye, thiocyanate, finish modifier, chemical sensitizers, and in finish time may be used as known in the art to reach an optimum finish position for a particular emulsion.

a. Melt emulsion at 40° C. Add 256 g of 12.5% gelatin solution (use limed ossein gelatin) to bring gel content to 78 g/mole silver.

b. Add 150 mg NaSCN. Hold 20 minutes with stirring.

c. Add green light spectral sensitizing dyes at 0.85 mmole dye/mole Ag. Higher or lower mole ratios may be employed in specific sensitizations. Single sensitizing dye or multiple sensitizing dye sensitizations may be employed as known in the art. When multiple dye sensitizations are employed the dyes may be added together or may be added separately with an optional hold time between additions.

d. Add 3.00 mg of sodium thiosulfate pentahydrate. Hold 2 minutes.

e. Add 1.50 mg of potassium tetrachloroaurate(III). Hold 2 minutes.

f. Add 40.0 mg finish modifier (3-(N-methylsulfonyl)-carbamoylethyl benzothiazolium tetrafluoroborate). Hold 15 minutes.

g. Raise melt temperature from 40 to 62.5 degrees over 13.5 minutes. Hold at 62.5 degrees for 22 minutes. Cool rapidly to 40 degrees and chill set with stirring.

#### EMULSION PRECIPITATION AND SENSITIZATION EXAMPLE 3

10 1. Starting kettle: 60° C., 25.0 g limed ossein gel, 55.0 g NaBr, 4872 g distilled water, 2 ml of Nalco-2341 Anti-foam.

2. Nucleation stage:

15 a. Double-jet nucleation with 2.5M AgNO<sub>3</sub> solution and 2.71M NaBr solution, both at 30 ml/min for three minutes. This is followed by a two-minute hold.

b. Adjust kettle pH with 35 ml of concentrated NH<sub>4</sub>OH (14.8M) diluted with 65 ml distilled water. Hold for 4 minutes.

20 c. Adjust pH back to starting value with HNO<sub>3</sub>. One minute hold.

d. Add to kettle 140 g limed ossein gelatin and 3866 g distilled water, melted together at 60° C. Hold two minutes.

25 3. Lateral growth: Double jet with pBr control at pBr = 1.39 at 60° C., using 2.5N AgNO<sub>3</sub> solution, and a salt solution which is 2.46M NaBr and 0.04M KI. Use a ramped flow rate profile, from 10 to 85 ml/min over

30 53.3 minutes. Stop the silver and salt flow, hold for 30 seconds.

4. pBr adjust segment: over 10 minutes, run 2.5N AgNO<sub>3</sub> at 40 ml/min, allowing the kettle pBr to shift to 3.26. When pBr = 3.26 is reached, control at 3.26 with a

35 2.5M NaBr solution.

5. Add 10 ml of solution containing 0.17 mg/ml potassium selenocyanate, diluted to 100 ml with distilled water. Hold 30 seconds.

6. Add 0.3 moles of KI dissolved in distilled water to

40 250 ml.

7. For 35 minutes, run 2.5N AgNO<sub>3</sub> at 40 ml/min. Allow the kettle pBr to shift to 3.26, then control at pBr 3.26 with 2.5M NaBr solution.

8. Wash emulsion to pBr = 3.11 using ultrafiltration, concentrate, add 260 grams of limed ossein gel, 80 ml of solution containing 0.34 mg/ml of 4-chloro-3,5-xylenol in methanol, chill set, and store.

45 The resulting emulsion was 1.7 microns equivalent circular diameter and 0.15 microns thick, with 3.6% iodide.

50 This procedure is representative of the green light spectral sensitizations on this emulsion type. Variations in sensitizing dye, thiocyanate, finish modifier, chemical sensitizers, and in finish time may be used as known in the art to reach an optimum finish position for a particular emulsion.

a. Melt emulsion at 40 C.

b. Add 100 mg NaSCN. Hold 20 minutes with stirring.

c. Add green light spectral sensitizing dyes at 0.9 mmole dye/mole Ag. Higher or lower mole ratios may be employed in specific sensitizations. Single sensitizing dye or multiple sensitizing dye sensitizations may be employed as known in the art. When multiple dye sensitizations are employed the dyes may be added together or may be added separately with an optional hold time between additions.

- d. Add 40.0 mg finish modifier (3-(N-methylsulfonyl)carbamoylethyl benzothiazolium tetrafluoroborate). Hold 15 minutes.
- e. Adjust melt pBr to 3.40 with dilute  $\text{AgNO}_3$ .
- f. Add 1.50 mg of potassium tetrachloroaurate(III). Hold 2 minutes.
- g. Add 3.00 mg of sodium thiosulfate pentahydrate. Hold 2 minutes.
- g. Raise melt temperature from 40 to 65.0 degrees over 15.0 minutes. Hold at 65.0 degrees for 8 minutes. Cool rapidly to 40 degrees and chill set with stirring.

#### EMULSION PRECIPITATION AND SENSITIZATION EXAMPLE 4

1. Starting kettle: 65° C., total volume of 4.0 liters, with 5.0 g/L limed ossein gelatin and 11.0 g/L  $\text{NaBr}$ . No anti-foam was used.

##### 2. Nucleation stage:

a. Double-jet nucleation using 1.00M  $\text{AgNO}_3$  and 1.2M  $\text{NaBr}$  solutions, both at 82 ml/min. This is followed by a two-minute hold.

b. Adjust kettle pH with 25 ml of concentrated  $\text{NH}_4\text{OH}$  (14.8M) diluted with 76 ml of distilled water. Hold for 4 minutes.

c. Adjust pH back to starting value with  $\text{HNO}_3$ . One minute hold.

d. Add to kettle a 5-L solution containing 140 g of limed ossein gelatin at 65° C. Hold 2 minutes.

3. Lateral growth: Double jet with pBr control at 1.55 at 65° C., using 2.5M  $\text{AgNO}_3$ , and a salt solution which is 2.46M  $\text{NaBr}$  and 0.04M KI. Use a ramped flow rate profile, from 8 to 82 ml/min over 53.5 minutes.

4. pBr adjust segment: over 10 minutes, run 2.5N  $\text{AgNO}_3$  at 40 ml/min, allowing the kettle pBr to reach 3.20. When pBr 3.20 is reached, control pBr at 3.20 with a 2.5M  $\text{NaBr}$  solution.

5. Add 0.3 moles of KI dissolved in distilled water to 200 ml.

6. For 5 minutes, run 2.5N  $\text{AgNO}_3$  at 40 ml/min, allowing the kettle pBr to shift to 3.20, then control at pBr=3.20 with 2.5M  $\text{NaBr}$  solution.

7. Continue double jet silver and salt for 20 minutes, except using a 2.5M  $\text{NaBr}$  solution which contains 100 mg  $\text{Na}_3\text{Fe}(\text{CN})_6$ .

8. Continue double jet silver and salt for 10 minutes, using 2.5M  $\text{NaBr}$ .

9. After lowering the temperature to 50° C., add 2.5M  $\text{NaBr}$  to the kettle to adjust the pBr to 2.62. Wash the emulsion to pBr=3.25 using ultrafiltration, concentrate, add 260 g of limed ossein gel, 80 ml of solution containing 0.34 mg/ml of 4-chloro-3,5-xylenol in methanol, chill set and store.

The resulting emulsion was 1.9 microns equivalent circular diameter and 0.143 microns thick, with 3.6% iodide.

This procedure is representative of the red light spectral sensitizations on this emulsion type. Variations in sensitizing dye, thiocyanate, finish modifier, chemical sensitizers, and in finish time may be used as known in the art to reach an optimum finish position for a particular emulsion.

a. Melt emulsion at 40° C. Add 256 g of 35.0% gelatin solution (use limed ossein gelatin) to bring gel content to 77 g/mole silver.

b. Add 150 mg  $\text{NaSCN}$ . Hold 20 minutes with stirring.

c. Add red light spectral sensitizing dyes at 1.0 mmole dye/mole Ag. Higher or lower mole ratios may be

employed in specific sensitizations. Single sensitizing dye or multiple sensitizing dye sensitizations may be employed as known in the art. When multiple dye sensitizations are employed the dyes may be added together or may be added separately with an optional hold time between additions.

d. Add 3.50 mg of sodium thiosulfate pentahydrate. Hold 2 minutes.

e. Add 1.75 mg of potassium tetrachloroaurate(III). Hold 2 minutes.

f. Add 40.0 mg of finish modifier (3-(N-methylsulfonyl)-carbamoylethyl benzothiazolium tetrafluoroborate). Hold 15 minutes.

g. Raise melt temperature from 40 to 65.0 degrees over 15.0 minutes. Hold at 65.0 degrees for 5 minutes. Cool rapidly to 40 degrees and chill set with stirring. Add additional heat to the emulsion by melting at 40° C., increase melt temperature from 40° to 65° C. over 15 minutes, hold for 15 minutes, and chill set with stirring.

#### PHOTOGRAPHIC EXAMPLE 1

A photographic recording material (Photographic Sample 1) was prepared by applying the following layers in the given sequence to a transparent cellulose triacetate support. The quantities of silver halide are given in g of silver per  $\text{m}^2$ . The quantities of other materials are in g per  $\text{m}^2$ .

Layer 1 {Antihalation Layer} black colloidal silver sol containing 0.236 g of silver, with 2.44 g of gelatin.

Layer 2 {Photographic Layer} Green sensitized silver iodobromide emulsion [6.3 mol % iodide, average grain diameter 0.52 microns, conventional morphology] at 1.61 g, cyan dye-forming image coupler C-2 at 0.73 g with gelatin at 3.23 g.

Layer 3 {Protective Layer} Gelatin at 3.23 g.

The film was hardened at coating with 2% by weight to total gelatin of hardner S-1. Surfactants, coating aids, scavengers and stabilizers were added to the various layers of this sample as is commonly practiced in the art. The image coupler was dispersed in an equal weight of dibutyl phthalate.

Photographic Sample 2 was prepared like Photographic Sample 1 except that 0.13 g of DIR compound D-3 was added to layer 2.

Photographic Samples 3 and 4 were prepared like Photographic Samples 1 and 2 respectively except that the silver halide emulsion in layer 2 was replaced by an equal weight of a green sensitized silver iodobromide emulsion [6 mol % iodide, average grain diameter 2.3 microns, average grain thickness 0.11 microns].

Photographic Samples 11-14 were prepared like Photographic Samples 1-4 except that 0.043 g of ballasted green absorber dye MD-1 was added to layer 3.

Photographic Samples 1-14 were exposed using white light to sinusoidal patterns to determine the Modulation Transfer Function (MTF) Percent Response as a function of spatial frequency in the film plane. Specific details of this exposure-evaluation cycle can be found at R. L. Lamberts and F. C. Eisen, "A System for the Automated Evaluation of Modulation Transfer Functions of Photographic Materials", in the *Journal of Applied Photographic Engineering*, Vol. 6, pages 1-8, February, 1980. A more general description of the determination and meaning of MTF Percent Response curves can be found in the articles cited within this reference. The exposed samples were developed generally according to the C-41 Process as described in the *British Journal of Photography Annual* for 1988 at pages 196-198.

The bleaching solution composition was modified so as to comprise 1,3-propylene diamine tetraacetic acid. The exposed and processed samples were evaluated to determine the MTF Percent Response as a function of spatial frequency in the film plane as described above.

bromide emulsion [4 mol % iodide, average grain diameter 1.1 microns, average thickness 0.12 microns] at 0.65 g, magenta dye-forming image coupler M-1 at 0.022 g, agents dye-forming image coupler M-2 at 0.51 g, DIR compound D-2 at 0.007 g, DIR compound D-3 at 0.022

TABLE 1

| Sample <sup>a</sup> | Emulsion <sup>b</sup> | Type | Dye  | DIR <sup>d</sup> | MTF Percent Response <sup>e</sup> |        |         |         |
|---------------------|-----------------------|------|------|------------------|-----------------------------------|--------|---------|---------|
|                     |                       |      |      |                  | 2.5 c/mm                          | 5 c/mm | 50 c/mm | 80 c/mm |
| 1C                  | C                     | N    | none | 98               | 98                                | 51     | 30      |         |
| 11C                 | C                     | Y    | none | 98               | 98                                | 56     | 32      |         |
| 3C                  | T                     | N    | none | 102              | 100                               | 78     | 58      |         |
| 13I                 | T                     | Y    | none | 103              | 107                               | 84     | 58      |         |
| 2C                  | C                     | N    | D-3  | 117              | 120                               | 80     | 58      |         |
| 12C                 | C                     | Y    | D-3  | 118              | 123                               | 86     | 60      |         |
| 4C                  | T                     | N    | D-3  | 120              | 125                               | 103    | 80      |         |
| 14I                 | T                     | Y    | D-3  | 123              | 130                               | 117    | 93      |         |

<sup>a</sup>Samples are identified as comparative (C) or inventive (I).

<sup>b</sup>Emulsions are identified as conventional morphology (C) or High Aspect Ratio Tabular morphology (T).

<sup>c</sup>Presence (Y) or absence (N) of a spatially fixed absorber dye positioned between the sensitized silver halide emulsion layer and the image exposure source.

<sup>d</sup>Presence and identity of DIR compound in the photographic material@

<sup>e</sup>MTF Percent Response as a function of spatial frequency in the film plane for the photographic material.

As is readily apparent on examination of the photographic data shown in Table 1, the samples incorporating both the High Aspect Ratio Tabular Grain silver halide emulsions and the spatially fixed absorber dye show a larger improvement in MTF Percent Response than would have been anticipated based on the performance of the comparative samples. An even larger improvement in MTF Percent Response unexpectedly occurs when a DIR compound is additionally present.

#### PHOTOGRAPHIC EXAMPLE 2

A color photographic recording material (Photographic Sample 101) for color negative development was prepared by applying the following layers in the given sequence to a transparent support of cellulose triacetate. The quantities of silver halide are given in g of silver per m<sup>2</sup>. The quantities of other materials are given in g per m<sup>2</sup>. All silver halide emulsions were stabilized with 2 grams of 4-hydroxy-6-methyl-1,3,3a,7-tetraazaindene per mole of silver.

Layer 1 {Antihalation Layer} black colloidal silver sol containing 0.236 g of silver, with 2.44 g of gelatin.

Layer 2 {First (less) Red-Sensitive Layer} Red sensitized silver iodobromide emulsion [3.9 mol % iodide, average grain diameter 0.6 microns, average grain thickness 0.09 micron] at 0.54 g, red sensitized silver iodobromide emulsion [4.2 mol % iodide, average grain diameter 1.7 microns, average grain thickness 0.08 micron] at 0.43 g, cyan dye-forming image coupler C-1 at 0.54 g, DIR compound D-1 at 0.017 g, BAR compound B-1 at 0.016 g, with gelatin at 1.61 g.

Layer 3 {Second (more) Red-Sensitive Layer} Red sensitized silver iodobromide emulsion [4.2 mol % iodide, average grain diameter 2.1 microns, average grain thickness 0.09 microns] at 1.13 g, cyan dye-forming image coupler C-2 at 0.23 g, DIR compound D-1 at 0.023 g, BAR compound B-1 at 0.005 g, cyan dye-forming masking coupler CM-1 at 0.032 g with gelatin at 1.61 g.

Layer 4 {Interlayer} Oxidized developer scavenger S-1 at 0.054 g, yellow dye material YD-1 at 0.12 g and 1.29 g of gelatin.

Layer 5 {First (less) Green-Sensitive Layer} Green sensitized silver iodobromide emulsion [3.9 mol % iodide, average grain diameter 0.6 microns, average thickness 0.09 microns] at 0.43 g, green sensitized silver iodo-

g magenta dye-forming masking coupler MM-1 at 0.043 g with gelatin at 1.88 g.

Layer 6 {Second (more) Green-Sensitive Layer} Green sensitized silver iodobromide emulsion [4.2 mol % iodide, average grain diameter 2 microns, average grain thickness 0.08 microns] at 1.08 g, magenta dye-forming image coupler M-1 at 0.043 g, magenta dye-forming image coupler M-2 at 0.13 g, magenta dye-forming masking coupler MM-1 at 0.022 g, DIR compound D-2 at 0.007 g, DIR compound D-3 at 0.008 g with gelatin at 1.08 g.

Layer 7 {Interlayer} Oxidized developer scavenger S-1 at 0.054 g, yellow colloidal silver at 0.032 g with 1.61 g of gelatin.

Layer 8 {First (less) Blue-Sensitive Layer} Blue sensitized silver iodobromide emulsion [4 mol % iodide, average grain diameter 0.1 microns, average grain thickness 0.09 micron] at 0.32 g, blue sensitized silver iodobromide emulsion [4 mol % iodide, average grain diameter 1.3 microns, average grain thickness 0.09 micron] at 0.16 g, yellow dye-forming image coupler Y-1 at 0.91 g, DIR compound D-4 at 0.04 g, BAR compound B-2 at 0.016 g with gelatin at 1.61 g.

Layer 9 {Second (more) Blue-Sensitive Layer} Blue sensitized silver iodobromide emulsion [3 mol % iodide, average grain diameter 2.6 microns, average grain thickness 0.12 microns] at 0.75 g, yellow dye-forming image coupler Y-1 at 0.22 g, DIR compound D-4 at 0.039 g, with gelatin at 1.21 g.

Layer 10 {Protective Layer} 0.108 g of dye UV-1, 0.118 g of dye UV-2, unsensitized silver bromide Lippman emulsion at 0.108 g, with gelatin at 0.89 g.

This film was hardened at coating with 2% by weight to total gelatin of hardner H-1. Surfactants, coating aids, scavengers, dyes and stabilizers were added to the various layers of this sample as is commonly practiced in the art.

Photographic Sample 102 was prepared like Photographic Sample 101 except that 0.02 g of ballasted red absorber dye CD-1 was added to layer 10.

Photographic Sample 103 was prepared like Photographic Sample 101 except that the emulsion employed in layer 3 was replaced by an equal quantity of an emul-

sion with an average grain diameter of 1.9 microns and an average grain thickness of 0.14 microns.

Photographic Sample 104 was prepared like Photographic Sample 103 except that 0.02 g of ballasted red absorber dye CD-1 was added to layer 10.

Photographic Sample 105 was prepared like Photographic Sample 103 except that the emulsion employed in layer 6 was replaced by an equal quantity of an emulsion with an average grain diameter of 1.7 microns and an average grain thickness of 0.15 microns.

Photographic Sample 106 was prepared like Photographic Sample 105 except that 0.02 g of ballasted red absorber dye CD-1 was added to layer 10.

Photographic Sample 107 was prepared like Photographic Sample 101 except that the emulsion employed in layer 6 was replaced by an equal quantity of an emulsion with an average grain diameter of 1.7 microns and an average grain thickness of 0.15 microns.

Photographic Sample 108 was prepared like Photographic Sample 107 except that 0.02 g of ballasted red absorber dye CD-1 was added to layer 10.

Photographic Sample 109 was prepared in a manner analogous to Photographic Sample 101 by applying the following layers in the given sequence to a transparent support of cellulose triacetate.

Layer 1 {Antihalation Layer} black colloidal silver sol containing 0.236 g of silver, with 2.44 g gelatin.

Layer 2 {First (less) Red-Sensitive Layer} Red sensitized silver iodobromide emulsion [3.9 mol % iodide, average grain diameter 0.73 microns, average grain thickness 0.09 micron] at 0.70 g, cyan dye-forming image coupler C-1 at 0.61 g, DIR compound D-3 at 0.039 g, BAR compound B-1 at 0.016 g, with gelatin at 1.61 g.

Layer 3 {Second (more) Red-Sensitive Layer} Red sensitized silver iodobromide emulsion [4 mol % iodide, average grain diameter 1.9 microns, average grain thickness 0.09 microns] at 0.65 g, cyan dye-forming image coupler C-2 at 0.33 g, DIR compound D-3 at 0.013 g, BAR compound B-1 at 0.016 g with gelatin at 1.15 g.

Layer 4 {Interlayer} Oxidized developer scavenger S-1 at 0.054 g, ballasted absorber dye MD-1 at 0.02 g and 0.65 g of gelatin.

Layer 5 {First (less) Green-Sensitive Layer} Green sensitized silver iodobromide emulsion [3.9 mol % iodide, average grain diameter 0.8 microns, average thickness 0.09 microns] at 0.52 g, magenta dye-forming image coupler M-1 at 0.38 g, magenta dye-forming image coupler M-2 at 0.13 g, DIR compound D-3 at 0.03 g with gelatin at 1.16 g.

Layer 6 {Second (more) Green-Sensitive Layer} Green sensitized silver iodobromide emulsion [4.2 mol % iodide, average grain diameter 1.9 microns, average grain thickness 0.08 microns] at 0.65 g, magenta dye-forming image coupler M-1 at 0.097 g, magenta dye-forming image coupler M-2 at 0.032 g, DIR compound D-3 at 0.007 g, DIR compound D-3 at 0.04 g with gelatin at 0.97 g.

Layer 7 {Interlayer} Oxidized developer scavenger S-1 at 0.054 g, yellow colored magenta dye-forming masking coupler MM-2 at 0.15 g with 0.65 g of gelatin.

Layer 8 {First (less) Blue-Sensitive Layer} Blue sensitized silver iodobromide emulsion [4 mol % iodide, average grain diameter 0.9 microns, average grain thickness 0.09 micron] at 0.43 g, yellow dye-forming image coupler Y-1 at 1.07 g, DIR compound D-4 at 0.043 g, with gelatin at 1.61 g.

Layer 9 {Second (more) Blue-Sensitive Layer} Blue sensitized silver iodobromide emulsion [3 mol % iodide, average grain diameter 3.2 microns, average grain thickness 0.10 microns] at 0.59 g, yellow dye-forming image coupler Y-1 at 0.43 g, DIR compound D-4 at 0.033 g, with gelatin at 1.21 g.

Layer 10 {Protective Layer 1} Gelatin at 1.61 g.

Layer 11 {Protective Layer 2} Gelatin at 0.71 g.

Photographic Sample 110 was prepared like Photographic Sample 109 except that 0.02 g of ballasted red absorber dye CD-1 was added to layer 10 and 0.02 g of ballasted green absorber dye MD-1 was omitted from layer 4 and added to layer 10.

Photographic Sample 111 was prepared in a manner analogous to that used to prepare Photographic Sample 101 by applying the following layers in the given sequence to a transparent support of cellulose triacetate.

Layer 1 {Antihalation Layer} black colloidal silver sol containing 0.236 g of silver, with 2.44 g gelatin.

Layer 2 {First (less) Red-Sensitive Layer} Red sensitized silver iodobromide emulsion [4.8 mol % iodide, average grain diameter 0.26 microns, conventional morphology] at 0.43 g, red sensitized silver iodobromide emulsion [6.1 mol % iodide, average grain diameter 0.5

25 microns, conventional morphology] at 1.29 g, cyan dye-forming image coupler C-1 at 0.62 g, DIR compound D-5 at 0.011 g, DIR compound D-6 at 0.018 g with gelatin at 2.1 g.

Layer 3 {Second (more) Red-Sensitive Layer} Red sensitized silver iodobromide emulsion [6.0 mol % iodide, average grain diameter 0.8 microns, conventional morphology] at 1.08 g, cyan dye-forming image coupler C-1 at 0.19 g, DIR compound D-5 at 0.022 g, DIR compound D-1 at 0.038 g, cyan dye-forming masking coupler CM-1 at 0.064 g with gelatin at 1.22 g.

Layer 4 {Interlayer} Oxidized developer scavenger S-2 at 0.16 g, and 0.65 g of gelatin.

Layer 5 {First (less) Green-Sensitive Layer} Green sensitized silver iodobromide emulsion [4.8 mol % iodide, average grain diameter 0.26 microns, conventional morphology] at 0.95 g, green sensitized silver iodobromide emulsion [6.4 mol % iodide, average grain diameter 0.5 microns, conventional morphology] at 0.77 g, magenta dye-forming image coupler M-3 at 0.48 g, DIR compound D-2 at 0.014 g, magenta dye-forming masking coupler MM-1 at 0.09 g with gelatin at 2.18 g.

Layer 6 {Second (more) Green-Sensitive Layer} Green sensitized silver iodobromide emulsion [12 mol % iodide, average grain diameter 0.8 microns, conventional morphology] at 1.08 g, magenta dye-forming image coupler M-3 at 0.34 g, magenta dye-forming masking coupler MM-1 at 0.044 g, DIR compound D-2 at 0.011 g with gelatin at 1.15 g.

Layer 7 {Interlayer} Gelatin at 0.43 g.

Layer 8 {Interlayer} Oxidized developer scavenger S-2 at 0.08 g, yellow colloidal silver at 0.067 g with 0.43 g of gelatin.

Layer 9 {First (less) Blue-Sensitive Layer} Blue sensitized silver iodobromide emulsion [4.8 mol % iodide, average grain diameter 0.3 microns, conventional morphology] at 0.17 g, blue sensitized silver iodobromide emulsion [6 mol % iodide, average grain diameter 0.6 microns, conventional morphology] at 0.37 g, yellow dye-forming image coupler Y-2 at 1.29 g, DIR compound D-7 at 0.1 g, with gelatin at 1.61 g.

Layer 10 {Second (more) Blue-Sensitive Layer} Blue sensitized silver iodobromide emulsion [9 mol % iodide, average grain diameter 0.9 microns, conventional mor-

phology] at 0.65 g, yellow dye-forming image coupler Y-2 at 0.19 g, DIR compound D-7 at 0.086 g, with gelatin at 0.70 g.

Layer 11 {Protective Layer 1} UV protective dye UV-1 at 0.066 g, UV protective dye UV-2 at 0.11 g

5

unsensitized silver bromide Lippman emulsion at 0.21 g, with gelatin at 0.54 g.

Layer 12 {Protective Layer 2} Gelatin at 0.89 g.

Photographic Sample 112 was prepared like Photographic Sample 111 except that 0.02 g of ballasted red absorber dye CD-1 was added to layer 11.



-continued



D-1



D-2



D-3



D-4



-continued  
D-5



D-6



B-1



S-1



S-2



UV-1



IV.2



41

Polymer Latex A: n-butyl acrylate/2-acrylamido-2-methylpropane sulfonic acid/2-acetoacetoxyethyl methacrylate (88:5:7)  $T_g = -28^\circ\text{C}$ .

**Polymer Latex C:** Methyl acrylate/2-acrylamido-2-methylpropane sulfonic acid/2-acetoacetoxyethyl methacrylate (91:5:4)  $T_g = +10.5^\circ\text{C}$ .

The Photographic Samples were exposed using white light to sinusoidal patterns to determine the Modulation Transfer Function (MTF) Percent Response as a function of spatial frequency in the film plane. Specific de-

tails of this exposure—evaluation cycle can be found at R. L. Lamberts and F. C. Eisen, "A System for the Automated Evaluation of Modulation Transfer Functions of Photographic Materials", in the *Journal of Applied Photographic Engineering*, Vol. 6, pages 1-8, February 1980. A more general description of the determination and meaning of MTF Percent Response curves can be found in the articles cited within this reference. The exposed samples were developed and bleached

generally according to the C-41 Process as described in the *British Journal of Photography Annual* for 1988 at pages 196-198. The bleaching solution composition was modified so as to comprise 1,3-propylene diamine tetra-acetic acid. The exposed and processed samples were evaluated to determine the MTF Percent Response as a function of spatial frequency in the film plane as described above.

Table 2 (below) lists the MTF Percent Response characteristics of the cyan dye images formed by the red light sensitive layers of the described photographic samples.

morphology emulsions on inclusion of the ballasted absorber dye (samples 111 and 112).

#### PHOTOGRAPHIC EXAMPLE 3

Photographic Samples 109 and 110 both include a ballasted green light absorber dye. In sample 109, the green light sensitive layers are positioned between the ballasted absorber dye and the exposing light source while in sample 110, the ballasted absorber dye is positioned between the green light sensitive layers and the exposing light source.

These samples were treated in the manner described

TABLE 2

| Sample <sup>a</sup> | MTF Percent Response of the Red Light Sensitive Layers as a Function of Film Formulation |                              |                              |          |        |         |         |
|---------------------|------------------------------------------------------------------------------------------|------------------------------|------------------------------|----------|--------|---------|---------|
|                     | Tabular<br>(A)                                                                           | Emulsion <sup>b</sup><br>(B) | Absorber <sup>c</sup><br>Dye | 2.5 c/mm | 5 c/mm | 50 c/mm | 80 c/mm |
| 101 C               | 2.0 × 0.08                                                                               | 2.1 × 0.09                   | No                           | 99       | 96     | 34      | 19      |
| 102 I               | 2.0 × 0.08                                                                               | 2.1 × 0.09                   | Yes                          | 103      | 101    | 36      | 19      |
| 103 C               | 2.0 × 0.08                                                                               | 1.9 × 0.14                   | No                           | 101      | 100    | 39      | 19      |
| 104 I               | 2.0 × 0.08                                                                               | 1.9 × 0.14                   | Yes                          | 102      | 104    | 42      | 26      |
| 105 C               | 1.7 × 0.15                                                                               | 1.9 × 0.14                   | No                           | 102      | 102    | 44      | 25      |
| 106 I               | 1.7 × 0.15                                                                               | 1.9 × 0.14                   | Yes                          | 103      | 105    | 45      | 25      |
| 107 C               | 1.7 × 0.15                                                                               | 2.1 × 0.09                   | No                           | 99       | 100    | 36      | 19      |
| 108 I               | 1.7 × 0.15                                                                               | 2.1 × 0.09                   | Yes                          | 101      | 101    | 41      | 21      |
| 109 C               | 1.9 × 0.08                                                                               | 1.9 × 0.09                   | No                           | 100      | 101    | 46      | 30      |
| 110 I               | 1.9 × 0.08                                                                               | 1.9 × 0.09                   | Yes                          | 105      | 105    | 47      | 33      |
| 111 P               | 0.8                                                                                      | 0.8                          | No                           | 100      | 99     | 25      | 9       |
| 112 P               | 0.8                                                                                      | 0.8                          | Yes                          | 101      | 100    | 26      | 9       |

<sup>a</sup>Samples are identified as comparison (C), inventive (I), or prior art (P).

<sup>b</sup>Dimensions of tabular grain AgX emulsions as average equivalent circular diameter × thickness (both in microns) in the most green sensitive layer (A) and the most red sensitive layer (B). For the conventional emulsions employed in the prior art comparisons, the equivalent circular diameter only is shown.

<sup>c</sup>Presence of red light absorbing ballasted absorber dye positioned between the most red light sensitive layer and the source of the imaging exposure.

<sup>d</sup>MTF Percent Response at the indicated spatial frequency in the film plane for the cyan dye images formed in the red light sensitive layers.

As can be readily appreciated on examination of the data presented in Table 2, the photographic samples incorporating both a tabular grain emulsion in the most light sensitive layer sensitized to a particular color, and

above (in Photographic Example 2) but were evaluated for MTF Percent Response in the magenta dye record formed by the green light sensitive layers. The results of this evaluation are shown below in Table 3.

TABLE 3

| Sample <sup>a</sup> | MTF Percent Response of the Green Light Sensitive Layers as a Function of Film Formulation |                              |                              |          |        |         |         |
|---------------------|--------------------------------------------------------------------------------------------|------------------------------|------------------------------|----------|--------|---------|---------|
|                     | Tabular<br>(A)                                                                             | Emulsion <sup>b</sup><br>(B) | Absorber <sup>c</sup><br>Dye | 2.5 c/mm | 5 c/mm | 50 c/mm | 80 c/mm |
| 109 C               | 1.9 × 0.08                                                                                 | 1.9 × 0.09                   | No                           | 100      | 101    | 46      | 30      |
| 110 I               | 1.9 × 0.08                                                                                 | 1.9 × 0.09                   | Yes                          | 105      | 105    | 47      | 33      |

<sup>a</sup>Samples are identified as comparison (C), or inventive (I).

<sup>b</sup>Dimensions of tabular grain AgX emulsions as average equivalent circular diameter × thickness (both in microns) in the most green sensitive layer (A) and the most red sensitive layer (B).

<sup>c</sup>Presence of green light absorbing ballasted absorber dye positioned between the most green light sensitive layer and the source of the imaging exposure.

<sup>d</sup>MTF Percent Response at the indicated spatial frequency in the film plane for the magenta dye images formed in the green light sensitive layers.

a ballasted absorber dye positioned between that most light sensitive layer and the source of the imaging exposure exhibit the largest MTF Percent Response within each sample pair that differ only by the presence or absence of the incorporated ballasted absorber dye (samples 101 and 102; 103 and 104; 105 and 106; 107 and 108; and 109 and 110).

These improvements in MTF Percent Response occur at both low and high spatial frequencies.

Additionally, the magnitude of the improvement in sharpness shown in the inventive samples vs their respective comparison samples on inclusion of the ballasted absorber dye is surprisingly larger than that observed in the prior art films incorporating conventional

As can be appreciated on examination of the photographic data presented in Table 3, the improvement in MTF Percent Response occurs in a green light sensitive element as a function of placing the green light absorbing dye between the imaging exposure source and the green light sensitive element. The improvements occur at both low and high spatial frequencies and are again larger in magnitude than those shown by the prior art comparisons included in Table 2.

The invention has been described in detail with particular reference to preferred embodiments thereof, but it will be understood that variations and modifications can be effected within the spirit and scope of the invention.

We claim:

1. A color negative photographic recording material comprising a support bearing at least one photographic layer comprising a sensitized high aspect ratio tabular grain silver halide emulsion having an average aspect ratio of greater than 10 and at least one dye layer positioned between said silver halide layer and the upper surface of said recording material, said dye layer comprising a spatially fixed dye that absorbs light in the region of the spectrum to which the silver halide is sensitized, wherein said photographic material comprises a dye forming DIR coupler compound and colored masking couplers.

absorbs light in the same wavelength as each most sensitive layer.

4. The photographic recording material according to claim 1 wherein said high aspect ratio tabular grain has an aspect ratio of greater than 15.

5. The photographic recording material according to claim 1 wherein said dye layer comprising spatially fixed dye is located above all of the sensitized emulsion layers in said photographic recording material.

6. The photographic recording material according to claim 1 wherein said spatially fixed dye comprises at least one of member selected from the group



2. The recording material of claim 1 wherein said photographic recording material comprises a support bearing at least three photographic elements, each photographic element being sensitized to different regions of the spectrum.

3. The photographic recording material according to claim 2 wherein more than one of the photographic elements comprise most sensitive photographic layers comprising a sensitized high aspect ratio tabular grain silver halide emulsions and said at least one dye layer

60  
7. The photographic recording material of claim 1 wherein said spatially fixed dye is present in an amount of about 0.5 mg/m<sup>2</sup> to about 200 mg/m<sup>2</sup>.

8. The material of claim 1 wherein said silver halide comprises silver bromoiodide.

9. A process of forming a color negative image comprising providing a color negative recording material comprising a support bearing at least one photographic

layer comprising a sensitized high aspect ratio tabular grain silver halide emulsion having an average aspect ratio of greater than 10 and at least one dye layer positioned between said silver halide layer and the upper surface of said recording material, said dye layer comprising a spatially fixed dye that absorbs light in the region of the spectrum to which the silver halide is sensitized, exposing said color negative recording material to actinic radiation, contacting said color negative recording material with developing agent to reduce 10 pler. developable silver halide and oxidize the color develop-

ing agent, the oxidized color developing agent in turn reacts with coupler in said dye layer to yield dye, then contacting said color negative recording material with a bleach, a fixer or bleach-fix, washing and drying to yield a color negative.

10. The process of claim 9 wherein said color negative recording material comprises a DIR compound.

11. The process of claim 9 wherein said color negative material further comprises colored masking coupler.

\* \* \* \* \*

15

20

25

30

35

40

45

50

55

60

65